

1

2,785,973

## PRODUCTION AND PURIFICATION OF TITANIUM

Philipp Gross, Eton, and David Leon Levi, Chalfont St. Peter, England, assignors to Fulmer Research Institute Limited, Stoke Poges, England

No Drawing. Application August 19, 1952,  
Serial No. 305,292

Claims priority, application Great Britain  
September 5, 1951

5 Claims. (Cl. 75—84.4)

It is known that impure metallic titanium can be made by the reduction of titania (either pure, or in a naturally occurring impure form such as rutile) for example by carbon using an electric furnace. The impurities in the product, however, especially carbon which may be present in substantial amounts, usually as carbide, and/or oxygen, cause it to be brittle and hence of little use in practice. Similarly if the raw material used for the reduction by carbon or any other reducing agent contains a titaniferous ore, an impure titanium alloyed with other metallic constituents, for example, iron and silicon, is formed, also having properties so much inferior to those of substantially pure titanium that its usefulness in metallurgical practice is very restricted.

Stahler and Bachran (Ber. deutsche chem. Ges. 44 (1911), 2907) formed metallic titanium by the thermal decomposition of titanium dichloride, titanium tetrachloride vapour being formed simultaneously; while the corresponding reaction with titanium dibromide was observed by Young and Schumb (J. Amer. Chem. Soc., 52 (1930), 4233). These dihalides were themselves formed by thermal decomposition at somewhat lower temperatures of the solid trichloride and tribromide respectively, likewise with the simultaneous formation of titanium tetrachloride and tetrabromide respectively. Klemm and Grimm (Zeits. anorg. chem. 249 (1942), 198) converted metallic titanium to a mixture of condensed lower titanium chlorides by reaction in a sealed tube with titanium tetrachloride, and Young and Schumb (J. Amer. Chem. Soc. 52 (1930), 4233) carried out a similar reaction with titanium and titanium tetrabromide. Meyer, Bauer and Schmidt (Ber. deutsche chem. Ges. 56B (1923), 1908) in reducing titanium tetrachloride vapour with hydrogen so as to condense titanium trichloride, found that when titanium was placed in the gas stream to absorb excess hydrogen chloride, an increased yield was obtained, and that the condensate contained a proportion of titanium dichloride.

We have found that the normally stable lower chlorides or bromides, especially the dihalides, of titanium can be obtained in a convenient way and with a very high yield by the reaction of the corresponding tetrahalide vapour with heated titanium bearing material, preferably under reduced pressure, whereby the vapours of these lower halides are formed and can be condensed as solids in a cooler zone. When using the unsaturated tetrahalide vapour the lower halides are condensed entirely free from unreacted tetrahalide, if any, which unreacted halide is therefore suitable for further use. We have further found that the impurities usually contained in impure titanium such as carbon (usually as carbide), oxygen and also small amounts of other metals such as iron, do not react with the tetrahalide vapour under these conditions so that the lower halides obtained when using impure titanium or other titanium bearing materials are substantially free from such impurities. Thus by disproportioning these lower halides into metallic titanium and the tetra-

2

halide, pure titanium is produced from the titanium bearing material and the originally applied tetrahalide is recovered.

We have also found that the metallic titanium formed by this procedure, consisting of small discrete leaflets (flakes) can on account of its form very readily be submitted to further metallurgical processing, for example to pressing and sintering, and on this account has considerable advantages over other metallic titanium products, for example the "sponge" which is formed by the reduction of titanium tetrachloride with magnesium.

According to the present invention, therefore, pure metallic titanium can be extracted from titanium bearing material of the group consisting of impure titanium and titanium alloys (especially impure titanium or titanium alloys, such as ferrotitanium, made by reduction of a raw material with carbon) by passing over them titanium tetrachloride or titanium tetrabromide vapour at elevated temperatures and in an inert atmosphere, i. e. an atmosphere containing titanium halides either alone and if so under reduced pressure or mixed with an inert carrier gas, such as argon, whereby these halides react with the titanium-bearing material to give the vapour of the normally stable titanium di- and/or tri-chloride or bromide respectively, leading these vapours from the reaction zone into a separate and adjacent zone where they are cooled, whereby the lower halides mainly condense as solids, and also to a small extent disproportionate into metallic titanium which condenses and titanium tetrachloride or tetrabromide vapours respectively which vapours are led into a separate and cooler condenser (tetrahalide condenser). In a subsequent step the solid condensed di- and/or trichlorides or bromides are heated preferably in vacuo but otherwise under a partial pressure of titanium tetrachloride or tetrabromide respectively lower than their decomposition pressures into these tetrahalides at the prevailing temperature, whereby they decompose yielding metallic titanium and titanium tetrachloride or tetrabromide vapour respectively. If the decomposition is carried out using hydrogen as carrier gas, the metallic titanium may afterwards require heating in vacuum to remove absorbed hydrogen. The titanium tetrahalide formed is also led into a separate condenser preferably the tetrahalide condenser referred to above, so that the whole of the titanium tetrachloride or tetrabromide originally used may be re-applied for further extraction; alternatively, since the vapour pressures of the titanium tetrachloride or tetrabromide are high at moderately elevated temperatures, they may be recirculated in the gaseous state without previous condensation. Again, since the di- and tri-chlorides (or bromides) are highly hygroscopic solids it is usually advantageous, but not necessary, to use one converter for both condensing and decomposing the lower halides by carrying out the process in the same chamber (converter) but in two consecutive steps, in the first of which titanium tetrachloride or tetrabromide is led over the titanium bearing material and metallic titanium and lower titanium halides condensed in the converter by cooling, and in the second of which the converter is heated while the stream of gaseous reaction products is diverted from it, and the solid lower titanium chlorides (or bromides) thus decomposed. By having at least two converters which are alternately heated and cooled and correspondingly connected with and disconnected from the stream of tetrachloride or tetrabromide, a continuous extraction can be achieved using either continuous circulation of the tetrahalide without condensation, or alternatively condensing the tetrahalide and using at least two tetrahalide condensers serving alternately as condensers and evaporators.

The method may be illustrated by considering typical

reactions occurring in the extraction of titanium by means of titanium tetrachloride according to the method of the invention. In the primary reaction we have in general the following:



On cooling the gaseous di- and tri-chlorides condense, while any unchanged tetrachloride passes on to the still cooler tetrahalide condenser. If the condenser containing the lower chlorides is now heated to a suitable temperature and evacuated or swept out by a stream of inert gas, these halides will decompose to yield pure titanium metal and regenerate titanium tetrachloride, e. g.,



The process for the production of titanium from titanium bearing material of the group consisting of impure titanium and titanium alloys according to the invention, thus comprises the following steps, all carried out in an inert atmosphere; heating the titanium bearing material, evaporating a titanium tetrahalide of the group consisting of chloride and bromide, leading the vapour of said tetrahalide in an unsaturated state over the heated material, thereby to form a vapour mixture containing said tetrahalide and lower normally stable titanium halides, leading said vapour mixture to a cooler zone whereby the lower halides condense as solids except for a small amount which decomposes into tetrahalide vapour and purified titanium which condenses with the lower halides, reducing the tetrahalide pressure in said cooler zone to a value lower than the decomposition pressure of the lower halides while heating the condensate therein to a temperature below the temperature at which under applied pressure the halides will dissociate into metallic titanium and free halogen, thereby to decompose the condensed lower halides into purified metallic titanium and tetrahalide vapour, and re-using the tetrahalide from the condensation and decomposition steps for further extraction of titanium from the titanium bearing material.

In the primary reaction the extent of conversion of the tetrahalide to lower halides in the gas phase will vary according to the conditions of temperature and pressure employed, as will also the relative proportions of the different lower halides formed. Similarly, according to the reaction conditions the relative proportions of the lower halides in the solid condensate to one another will vary, in some cases one halide predominating, as for example the dichloride under the conditions described in the examples below. Both reactions are endothermic, so that the conversion into the lower halides will be higher at higher temperatures. The conversion is also dependent on the pressure the dihalide formation being relatively somewhat favoured by decreasing pressure. (See spec.)

In carrying out the process according to the invention, in order to ensure that the condensed solid lower titanium halides are pure and are not contaminated with small quantities of oxide or carbide or other impurities such as silicon or aluminum, it is of importance that these lower halides are condensed on a surface composed of materials which do not react with the lower halides to produce substances which bring about such contamination. The use of titanium and also of molybdenum, for example, has been found advantageous for this purpose. A suitable lining of titanium may also be formed on the surface of another refractory material, for example mullite or similar oxygen-containing materials, due to reaction between the lower titanium halides and the original surface of the refractory leading to the formation of a protective surface layer on which the lower titanium halides may be condensed without contamination. Graphite (or a refractory carbide) likewise provides a

suitable condenser material, protective coatings (of titanium carbide) being formed in this case also.

A suitable combination of temperature and pressure when using titanium tetrachloride according to the method of the invention may be seen from the following example. A stream of argon was saturated with titanium tetrachloride vapour at 20° C. (thus containing titanium tetrachloride at a partial pressure of about 10 mm.) and was passed over pieces of impure titanium (3 to 6 mesh), containing carbon as main impurity, maintained at about 1050° C. and contained in a graphite tube lined with a material, such as molybdenum, showing no reaction with the gaseous products under these reaction conditions. The reaction products passed into a cooler zone of the tube where a condensate formed consisting mainly of titanium dichloride in yield corresponding to about 40% of complete conversion of tetrachloride, but containing also much smaller amounts of metallic titanium and titanium trichloride. The stream of argon containing titanium tetrachloride vapour was discontinued, a stream of pure argon passed and the temperature of the condensate raised to about 950° C. Titanium tetrachloride vapour was evolved and collected in a suitable condenser, but after some time the argon stream leaving the reaction tube no longer contained titanium tetrachloride vapour, and metallic titanium, free from carbon, remained in the condenser.

In a similar experiment in which the partial pressure of titanium tetrachloride was 180 mms., and the impure titanium was maintained at 1050° C., the reaction products condensing again consisted mainly of titanium dichloride (in a yield corresponding to about 35% of complete conversion of the tetrachloride), together with much smaller amounts of titanium trichloride and metallic titanium. The lower chlorides were converted to metallic titanium by heating to 950° C. in the manner described above.

In similar experiments with titanium tetrabromide in which partial pressures of about 5 mms. and 80 mms. were used, and the impure titanium was maintained around 1000° C., the reaction products in the condenser consisted mainly of titanium dibromide which was obtained in good yield, together with minor amounts of titanium tribromide and metallic titanium. The reaction products were heated in a stream of pure argon at around 800° C., and the titanium tetrabromide evolved was collected in a suitable condenser. When decomposition of the lower halides was complete, metallic titanium free from carbon remained in the condenser.

We claim:

1. A process for extracting titanium from titanium bearing material of the group consisting of impure titanium and titanium alloys which comprises the following steps, all carried out in an inert atmosphere; heating the titanium bearing material, evaporating a titanium tetrahalide of the group consisting of chloride and bromide, leading the vapour of said tetrahalide in an unsaturated state over the heated material, thereby to form a vapour mixture containing said tetrahalide and lower normally stable titanium halides, leading said vapour mixture to a cooler zone whereby the lower halides condense as solids except for a small amount which decomposes into tetrahalide vapour and purified titanium which condenses with the lower halides, reducing the tetrahalide pressure in said cooler zone to a value lower than the decomposition pressure of the lower halides while heating the condensate therein to a temperature below the temperature at which under the applied pressure the halides will dissociate into metallic titanium and free halogen, thereby to decompose the condensed lower halides into purified metallic titanium and tetrahalide vapour, and re-using the tetrahalide from the condensation and decomposition steps for further extraction of titanium from the titanium bearing material.

2. A process for extracting titanium from titanium

bearing material of the group consisting of impure titanium and titanium alloys which comprises the following steps, all carried out in an inert atmosphere; heating the titanium bearing material, evaporating a titanium tetrahalide of the group consisting of chloride and bromide, leading the vapour of said tetrahalide in an unsaturated state and under a partial vacuum over the heated material thereby to form a vapour mixture containing said tetrahalide and lower normally stable titanium halides, leading said vapour mixture to a cooler zone whereby the lower halides condense as solids except for a small amount which decomposes into tetrahalide vapour and purified titanium which condenses with the lower halides, reducing the tetrahalide pressure in said cooler zone to a value lower than the decomposition pressure of the lower halides while heating the condensate therein to a temperature below the temperature at which under the applied pressure the halides will dissociate into metallic titanium and free halogen, thereby to decompose the condensed lower halides into purified metallic titanium and tetrahalide vapour, and re-using the tetrahalide from the condensation and decomposition steps for further extraction of titanium from the titanium bearing material.

3. A process for extracting titanium from titanium bearing material of the group consisting of impure titanium and titanium alloys which comprises the following steps, all carried out in an inert atmosphere; heating the titanium bearing material, evaporating a titanium tetrahalide of the group consisting of chloride and bromide, leading the vapour of said tetrahalide in an unsaturated state over the heated material, thereby to form a vapour mixture containing said tetrahalide and lower normally stable titanium halides, leading said vapour mixture to a cooler zone whereby the lower halides condense as solids except for a small amount which decomposes into tetrahalide vapour and purified titanium which condenses with the lower halides as flakes, reducing the tetrahalide pressure in said cooler zone to a value lower than the decomposition pressure of the lower halides while heating the condensate therein to a temperature below the temperature at which under the applied pressure the halides will dissociate into metallic titanium and free halogen, thereby to decompose the condensed lower halides into flakes of purified metallic titanium and tetrahalide vapour, and re-using the tetrahalide from the condensation and decomposition steps for further extraction of titanium from the titanium bearing material.

4. A process for extracting titanium from titanium bearing material of the group consisting of impure titanium and titanium alloys which comprises the following steps, all carried out in an inert atmosphere; heating the titanium bearing material, evaporating a titanium tetrahalide of the group consisting of chloride and bromide, leading the vapour of said tetrahalide in an unsaturated state over the heated material, thereby to form a vapour mixture containing said tetrahalide and lower normally stable titanium halides, leading said vapour mixture to a cooler zone whereby the lower halides condense as solids except for a small amount which decomposes into tetrahalide vapour and purified titanium which condenses with the lower halides, reducing the tetrahalide pressure

in said cooler zone to a value lower than the decomposition pressure of the lower halides while heating the condensate therein to a temperature below the temperature at which under the applied pressure the halides will dissociate into metallic titanium and free halogen, thereby to decompose the condensed lower halides into purified metallic titanium and tetrahalide vapour, leading the vapour from the condensation and decomposition steps into a still cooler zone to condense said tetrahalide, heating said condensate in said last named zone to re-evaporate said tetrahalide and using said tetrahalide vapour for further extraction of titanium from the titanium bearing material, at least two such still cooler zones being provided and used alternately as condenser and evaporator.

15 5. A process for extracting titanium from titanium bearing material of the group consisting of impure titanium and titanium alloys which comprises the following steps, all carried out in an inert atmosphere; heating the titanium bearing material, evaporating a titanium tetrahalide of the group consisting of chloride and bromide, leading the vapour of said tetrahalide in an unsaturated state over the heated material, thereby to form a vapour mixture containing said tetrahalide and lower normally stable titanium halides, leading said vapour mixture to a cooler zone whereby the lower halides condense as solids except for a small amount which decomposes into tetrahalide vapour and purified titanium which condenses with the lower halides, reducing the tetrahalide pressure in said cooler zone to a value lower than the decomposition pressure of the lower halides while heating the condensate therein to a temperature below the temperature at which under the applied pressure the halides will dissociate into metallic titanium and free halogen, thereby to decompose the condensed lower halides into purified metallic titanium and tetrahalide vapour, at least two such cooler zones being provided and used alternately as lower halide condensers and decomposers, and re-using the tetrahalide from the condensation and decompositon steps for further extraction of titanium from the titanium bearing material.

#### References Cited in the file of this patent

#### UNITED STATES PATENTS

|    |           |           |               |
|----|-----------|-----------|---------------|
| 45 | 1,046,043 | Weintraub | Dec. 3, 1912  |
|    | 2,670,270 | Jordan    | Feb. 23, 1954 |
|    | 2,706,153 | Glasser   | Apr. 12, 1955 |

#### OTHER REFERENCES

50 Deutsche Chemische Gesellschaft Berichte, Jahrig 44, Band 3. Oct. 9, Dec. 11, 1911. Pages 2906-2915.

A Comprehensive Treatise on Inorganic and Theoretical Chemistry by Mellor, vol. VII, page 74. Pub. 1927 by Longmans, Green & Co., 55 fifth Ave., N. Y.

55 Information Circular 7381, Nov. 1946, pages 5, 6. Pub. by Bureau of Mines, D. C.

Bureau of Mines Report of Investigations 4519. Pub. Aug. 1949 by Bureau of Mines, Dept. of Interior, Washington, D. C. Page 13.

60 Jordan, Abandoned application Serial No. 165,863, filed June 2, 1950.